

## 1

3,687,721

**POLYESTER MULTIFILAMENT YARNS**  
Kimon C. Dardoufas, Richmond, Va., assignor to  
Allied Chemical Corporation, New York, N.Y.  
No Drawing. Filed May 19, 1969, Ser. No. 825,987  
Int. Cl. B32b 27/06, 27/36

U.S. Cl. 117—138.8 F

3 Claims

### ABSTRACT OF THE DISCLOSURE

An improved multifilament yarn having a lubricating protective film allowing higher stretching for increased molecular orientation is prepared by applying to the yarn a liquid composition of about 0.4 to about 1.5 weight percent based on the weight of the yarn, said film composition comprising decaglycerol tetraoleate, glycerol monooleate, ethoxylated tall oil fatty acid, sulfated glycerol trioleate, ethoxylated alkylamine and a lubricant of hexadecyl stearate. Other additives, such as antioxidants may be added as well as the composition may be aqueous or nonaqueous.

### BACKGROUND OF THE INVENTION

This invention relates to improved multifilament yarns, and particularly to multifilament yarns for industrial uses. More particularly, it relates to a process for the treatment of multifilament yarns so as to improve their resistance to the degrading effect of exposure to heat and to aging.

In processing thermoplastic filaments, fibers, yarns and threads, some type of fluid treatment is usually required to maximize inter-filament cohesion during processing to accentuate operability during routine processing in manufacturing the yarn as well as for necessary subsequent operations. Various well known additives are also often added during the manufacture of the yarn in an effort to give better operability during the manufacture of the yarn as well as to give greater resistivity of the yarn to the deteriorating effects of heat and age.

The demands for industrial yarns having improved properties, such as greater strength not only when made but having the ability to retain the greater strength under strenuous industrial conditions, and greater resistivity of the yarn to the deteriorating effects of heat and age are increasing almost in direct proportion to the growth of industrial society.

The multifilament yarns applicable for use in the present invention are prepared from polyamides and polyesters or from copolymers or coblends thereof. The multifilament yarns particularly applicable for use in the present invention are prepared from polyester and polyamide. The former can be utilized in the present invention whether prepared either by the well known ester interchange reaction between dimethyl terephthalate and an alkylene glycol or the more recently improvised direct esterification process wherein terephthalic acid and an alkylene glycol under certain conditions can directly yield the synthetic linear polyesters from which the polyester yarns are prepared.

Many methods and compositions are known for the fluid treatment of textile materials; however, no method or composition is known that satisfies all the operational difficulties as well as yields a product having all the parameters necessary for a first quality grade industrial yarn. The age old problem of wettability, for example, has crept back into the problem area as higher-speed drawing of the yarn has evolved. As the yarn is passing over the fluid treatment surface at a speed substantially greater than heretofore, it becomes more difficult to maintain proper wettability.

A relatively heavy coating of fluid must necessarily be

## 2

applied to the yarn in order to give proper lubricity allowing greater molecular orientation during subsequent processing with consequent greater strength. A method and composition to allow proper wettability and lubricity is therefore necessary for the preparation of improved industrial yarns.

A textile treating fluid usually comprises lubricants, emulsifiers and antistats or wetting agents plus other ingredients necessary to assist in obtaining the desired textile material. Any one ingredient must of necessity interrelate in such a way with all the other ingredients so the overall treating fluid is compatible to the extent of having sufficient wetting ability and therefore give sufficient lubricity to the yarn.

For example, it has rarely been possible to obtain stable fully emulsified compositions containing greater than twenty-five percent solids and having viscosity sufficiently low for application to a textile material. If the viscosity of the emulsion is improper then the fluid cannot be uniformly spread over the yarn filaments in the short interval of time that the yarn is in contact with the fluid treating surface.

The emulsifiers must have a proper HLB value. The HLB value of an emulsifier is defined as their hydrophilic-lipophilic balance. HLB values of 1 to 10 are strongly attracted to the oil phase to be dispersed and are emulsification agents for oils and fats. Values above 10 are strongly attracted to water and are emulsification agents for the aqueous component. The determination of these and other values are made in accordance with the method depicted in the Kirk-Othmer Encyclopedia of Chemical Technology, vol. 8, 2nd edition, pages 117-154, John Wiley & Sons, 1965.

The antistat and/or wetting agent must be present in such an amount and be of such a composition as to be compatible with high-speed elongation to yield sufficient low static to avoid kick-back in the high-speed drawing apparatus thus permitting drawing of the yarn to sufficiently high-draw ratio to achieve necessary strength characteristics for first quality industrial yarn while maintaining minimal operation difficulties, such as, low wraps and breaks per pound.

Other necessary parameters of textile treating fluids are, for example, the fluid components, when deposited on the yarn, must be capable of resisting heat treatment of temperatures in the range of up to about 250° C. without volatilizing or significantly altering the lubricity, static and stability of the composition. The fluid ingredients, when applied to the yarn also must have low yarn to metal frictional characteristics to avoid abrasion and wearing of the processing equipment. Antioxidants may also be used with said fluid to assist in resisting aging and heat deterioration.

It has been observed that with higher speed processing necessary in the manufacturing of improved higher strength multifilament yarns that processing difficulties as well as inability to obtain the necessary quality yarn have made it necessary to explore other fluid treating methods and compositions in an effort to alleviate this problem. Therefore, an improved method and composition that would interrelate the ingredients of a fluid treating composition to allow substantial processing improvement and simultaneously obtain high quality yarn having a lubricating protective film allowing higher stretching for increased molecular orientation and having greater resistance to the degrading effect of exposure to heat and to aging would make a substantial contribution to this art.

### SUMMARY OF THE INVENTION

It is, therefore, a primary object of this invention to provide an improved multifilament yarn for use in indus-

try. Another object is to provide a novel textile treating composition for multifilament yarn. Still another object is to provide a novel textile treating composition which significantly improves processing difficulties upon its application to the yarn. A further object is to provide a novel textile treating composition that, upon its application to the yarn gives greater lubricity to said yarn. A still further object is to provide a novel textile treating composition that, upon its application to the yarn gives greater lubricity and allows higher stretching or drawing of the yarn for increased molecular orientation. Another object of the invention is to provide an improved multifilament yarn for industrial use having greater resistance to the degrading effect of exposure to heat and to aging. Still another object is to provide an improved process for preparing an improved multi-filament yarn for industrial use. Other objects will be apparent from time to time in the following specification.

These and other objects are attained in accordance with one mode of the present invention by providing for the manufacture of multifilament yarn to which has been applied about 0.4 to about 1.5 weight percent based on the weight of the yarn, of a liquid coating composition comprising about 13 to about 25 weight percent of said composition selected from the group consisting of glycerol monoleate and decaglycerol tetraoleate with ethoxylated tall oil fatty acids, about 12 to about 20 weight percent of said composition selected from the group consisting of sulfated glycerol trioleate and ethoxylated alkylamine, and about 55 to about 75 weight percent of said composition hexadecyl (isocetyl) stearate.

Another mode of the present invention is attained by providing for the manufacture of multifilament yarn to which has been applied about 0.4 to about 1.5 weight percent based on the weight of the yarn of a liquid coating composition comprising about 13 to about 25 weight percent of said composition selected from the group consisting of glycerol monoleate and decaglycerol tetraoleate with ethoxylated tall oil fatty acids, about 12 to about 20 weight percent of said composition selected from the group consisting of sulfated glycerol trioleate and ethoxylated alkylamine, about 55 to about 75 weight percent of said composition hexadecyl (isocetyl) stearate, and about 1 to about 3 weight percent of said composition of 4,4'-thiobis-(6-tert-butyl-m-cresol).

The lubricants suitable for use in the present invention are a branched chain alcohol combined with a fatty acid having 14 to 22 carbon atoms in the chain and having the general structural formula as indicated in Formula I,

Formula I



wherein  $n^1$ ,  $n^2$ , and  $n^3$  are independent integers and wherein  $n^1$  has a value of 4 to 10,  $n^2$  has a value of 6 to 12 and  $n^3$  has a value of 12 to 22. Preferably, the values of  $n^1$ ,  $n^2$  and  $n^3$  are  $5\pm 2$ ,  $7\pm 3$  and  $16\pm 3$  respectively. More preferably Formula I is hexadecyl stearate (isocetyl stearate) and still more preferably Formula I consists of about 45 weight percent of the above described stearate radical and about 55 weight percent palmitate radical. The amount of lubricant employed in the present invention may vary considerably but a preferred amount is about  $65\pm 20$  weight percent of the total solids content of the composition. This component is a liquid at 0°C. and has excellent hydrolytic and oxidative stability.

The esterified branched chain alcohol as shown in Formula I can be replaced with up to 50 weight percent with a triglyceride esterified with a fatty acid and then rear-

ranged. Such triglyceride has the general formula as indicated in Formula II,

Formula II



wherein  $y^1$ ,  $y^3$  and  $y^5$  are the number of carbon atoms in the fatty acid chain and are independent variable integers having a numerical value of 11 to 17, and  $x^2$ ,  $x^4$  and  $x^6$  are the number of hydrogen atoms in the fatty acid chain and are independent variable integers having a numerical value of 23 to 35. Preferably the triglyceride of the present invention should not exceed about 34 weight percent of the total solid. This component is a liquid at room temperature.

Emulsification agents are a most important constituent of the textile treating fluid composition. Suitable emulsification agents for use in the present invention are polymerized glycerol esterified with an unsaturated fatty acid having 14 to 20 carbon atoms in the chain and having the general formula as indicated in Formula III,

Formula III



wherein  $z^1$ ,  $z^3$ ,  $z^5$  and  $z^7$  are independent variable integers having a numerical value of 13 to 19 and wherein  $z^2$ ,  $z^4$ ,  $z^6$  and  $z^8$  are independent variable integers having a numerical value of 27 to 39, and further wherein at least 2 of the fatty acid chains contain at least 1 but not more than 3 double bonds, and still further wherein  $x^1$ ,  $x^2$ ,  $x^3$ ,  $x^4$  and  $x^5$  are either a fatty acid chain or hydrogen and are independently variable with each other.  $K^1$  has a numerical value of 4 to 10 glyceride units. This emulsifier composition has an HLB value of  $6.0\pm 1.0$ .

Other emulsification agents suitable for use in the present invention are hexaglycerol hexalaurate (HLB=6.0), hexaglycerol hexaoleate (HLB=5.0), sorbitan monopalmitate (HLB=6.7), hexaglycerol distearate (HLB=7.0), hexaglycerol trioleate (HLB=7.0), and decaglycerol tri-stearate (HLB=7.0) where at least 45 weight percent of the stearic acid portion of the ester employed has been replaced with oleic acid. The preferred component of the emulsification agent is decaglycerol tetraoleate having an HLB value of 6.0. This component of the emulsification agent is generally used in the amount of about 4 to 15 weight percent of the total solids. A second component of the emulsification agent is a glycerol esterified with an unsaturated fatty acid as indicated in Formula IV,

Formula IV



wherein  $z^1$  is the number of carbon atoms in the fatty acid chain and is an independent variable integer having a numerical value of 13 to 19 and  $z^2$  is the number of hydrogen atoms in the fatty acid chain and is an independent variable integer having a numerical value of 27 to 39.  $R^1$ ,  $R^2$  and  $R^3$  are selected from the group consisting of long chain fatty acids or hydrogen. In the preferred form, this component of the emulsification agent is 80 weight percent mono-oleate and 20 weight percent di-, tri- or unsubstituted glycerols. This component of the emulsification agent may be substituted with decaglycerol decaoleate (HLB=3.0), decaglycerol decalinoleate (HLB=3.0) and decaglycerol octaoleate (HLB=4.0). This preferred form of the component indicates a strong attraction for the oil phase of the emulsion. The third component of the emulsification agent is an ethoxylated tall oil which contains about 15 ethylene oxide units. This ethoxylated tall oil is subdivided into two major chemical groups. The first group is indicated as Formula A,

Formula A



wherein  $n$  is an independent variable integer having a numerical value of 10 to 20 and  $R'$  represents a long chain fatty aliphatic component acid having 13 to 19 carbon atoms and having 27 to 39 hydrogen atoms. The fatty acid constituents are selected from the group consisting of palmitic, linoleic and oleic acids which are condensed with a polyethylene oxide containing 10 to 20 moles of ethylene oxide. The first group represents about 60 weight percent of this component of the emulsification agent. The second group is indicated as Formula B and represents about 40 weight percent of this component of the emulsification agent,

Formula B



wherein  $n$  is an independent variable integer having a numerical value of 10 to 20 and  $R^2$  represents alicyclic resin acids which contain 50 to 60 weight percent of a mixture of abietic acid, dehydro abietic acid, levo pimamic acid, palustric acid, neoabietic acid, pimamic acid, isopimamic acid and other terpene acids in small quantities. The approximate preferred distribution in weight percent is as follows: Abietic (podocarpa-8,9-dien-15-oic, 13 isopropyl) acid=25-33, dehydro abietic (podocarpa-8,11,13-trien-15 oic, 13 isopropyl)=20-25, levo pimamic (podocarpa-8(14), 6-dien-15-oic, 13 isopropyl) and palustric (podocarpa-8, 13-dien-15-oic, 13 isopropyl) acid=8-12, neoabietic acid, pimamic acid, isopimamic acid and other terpene acids=small quantities that are substantially unremovable from the other major components of this group.

Other suitable replacements for the tall oil ethylene oxide composition are polyethylene oxides of sorbitan monoleate (HLB=9.0), polyoxyethylene sorbitan trioleate (HLB=11.0), polyoxyethylene sorbitol hexaoate (HLB=10.2), polyoxyethylene laurel ether (HLB=9.7). The tall oil composition containing abietic acid, dehydro abietic acid, levo pimamic acid and palustric acid is the preferred composition of this group as it yields the higher percentage of solids in the emulsions of the ethoxylated tall oil.

The preferred tall oil ethylene oxide composition makes up about 6 to 18 percent of the solids in the total finish composition. A lubricant HLB ratio can be determined by taking a weighted average HLB and multiplying this value times the weight percent of the lubricant of the total solids content and dividing by 100. The lubricant compositions having a lubricant HLB ratio of  $4.6 \pm .3$  have excellent emulsion stability.

The antistats and/or wetting agents suitable for use in the present invention are a glycerol condensed with unsaturated fatty acid sulfated to about 8 weight percent  $\text{SO}_3$  as indicated in Formula V,

Formula V



wherein  $n^1$ ,  $n^2$ ,  $n^3$ ,  $n^4$ ,  $n^5$  and  $n^6$  are independent integers having a numerical value of 5 to 9. Although lower sulfonation values may be employed, fully sulfated glycerol trioleate is preferable. This component besides being a good antistat and wetting agent also has emulsification properties and an HLB value of greater than 12. This component of the finish composition makes up about 9 to 13 weight percent of the solids in the total finish composition.

Other antistats and/or wetting agents suitable for use in the present invention are represented as shown in Formula VI,

25 Formula VI



wherein R is an alkyl chain of a fatty amine having 16 to 18 carbon atoms in the chain, and wherein  $x$  and  $y$  are independent variable integers having a numerical value of 8 to 12. Other long chain alkyl ethoxylated amines may be used provided they are liquid at room temperature and have antistatic properties. These ethoxylated alkyl amines have an HLB value of about 15.5. Further, they become cationic below 7.0 pH and are non-ionic above a pH of 7.0. The use of a mixture of the materials of Formula V and Formula VI being anionic and cationic respectively, results in synergistic increased antistatic properties. It is not understood at this time how this unusual phenomena works. It is clear, however, that a synergistic effect is obtained by measuring the HLB value as well as in actual use. For example, an over-all lubricity HLB ratio of  $6.8 \pm 0.3$  for the emulsification agents and antistat wetting agent yields an excellent emulsion stability.

The antioxidants suitable for use in the present invention, though not essential for good emulsification stability and good performance in the drawing operation, are 4,4'-thio - bis-(6-tert-butyl-m-cresol); 2,2<sup>1</sup> methylene bis(4-chlorophenol); 2-5, tertiary butyl hydroquinone; 6 dodecyl, 1,2 - dihydro 2,2,4 - trimethylquinoline; diphenylamine acetone; p-isopropoxy diphenylamine, thio-bis (di-sec.-amylphenol); trinonylphenyl phosphite and 9,9 dialkyl dihydroacridine. This component of the finish composition may be employed in an amount of 1 to 5 weight percent, preferably about 2 weight percent of the solids in the finish composition.

## PREFERRED EMBODIMENTS

60 The following examples specifically illustrates the manner in which the present invention is conducted and the advantages obtained thereby. The examples are illustrative only and are not to be construed as limitative.

## 65 Example 1

A series of finishes (A) through (I) are made up containing the ingredients as indicated in Table I. The ingredients are mixed together in the weight proportions as shown in Table I to form a concentrate. A small percentage of water is added to the concentrate until a clear solution is attained. Then, the concentrate is added slowly to water with good agitation of the aqueous solution to obtain a 35 weight percent as solids. In approximately 1/2 hour, excellent emulsion stability is obtained. Each solution is made up to contain 35 percent solids and 65

percent water. The emulsion stabilities are rated as excellent=no separations for a period of greater than 1 week; good=slight ring separation after 1 day; fair=less than 1 percent separation by volume after 24 hours; poor=over 1 percent separation by volume within 4 hours. Generally, it may be said that to have good commercial performance in a continuous spinning and drawing operation or

surface. The contact angles were measured with a refined version of the contact angle goniometer described in the Journal of Colloid Science 1, 513 (1946) by W. C. Bigelow, D. L. Pickett and W. A. Zisman.

5 From the contact angle data of Table II it can be seen that A, B, E, and H have the best wetting ability on polyester fiber.

TABLE II

Example Properties of Finishes in Table I

| Finish composition identity percent solids         | A 100     | B 100     | C 100 | D 100 | E 100 | F 100 | G 100 | H 100     | I 100    |
|----------------------------------------------------|-----------|-----------|-------|-------|-------|-------|-------|-----------|----------|
| Concentrate viscosities in cp. <sup>1</sup>        | 126       | 157       | 226   | 267   | 214   | 121   | 123   | 154       | 270      |
| Concentrate contact angles on polyester in degrees | 8.2       | 9.3       | 11.0  | 12.3  | 7.5   | 14.0  | 12.3  | 9.8       | 20.7     |
| Percent solids                                     | 35        | 35        | 35    | 35    | 35    | 35    | 35    | 35        | 35       |
| Percent water                                      | 65        | 65        | 65    | 65    | 65    | 65    | 65    | 65        | 65       |
| Emulsion viscosity in cp. <sup>1</sup>             | 10.7      | 10.6      | 15.8  | 16.7  | 7.0   | 10.6  | 15.5  | 7.7       | 27.2     |
| Emulsion contact angles on polyester in degrees    | 17.3      | 13.7      | 17.0  | 35.0  | 17.3  | 17.3  | 28.7  | 23.3      | 23.3     |
| Emulsion stability                                 | Excellent | Excellent | Good  | Fair  | Good  | Poor  | Fair  | Excellent | Solution |
| Overall lubricity HLB ratio                        | 6.8       | 6.9       | 5.6   | 5.4   | 5.4   | 5.6   | 6.7   |           |          |

<sup>1</sup> Centipoises

separate spinning operation and separate drawing of polyesters type fibers, the emulsions must rate excellent. The 20 concentrate should be clear. When diluted at 35 percent solids level with water, the emulsion must be essentially perfect or having no visible separation.

Prior to addition of water, the viscosity of 100 percent 25 concentrate of the various emulsions is measured using a Brookfield viscosimeter Model LVT device. This viscosity is measured in centipoises under standard conditions. An ultralow UL-adapter is employed for the viscosity measurement of emulsions which has its own spindle container and uses a #1 spindle. Since the emulsion and concentrate is Newtonian in character, viscosity can be determined directly at 25° C.

## Examples 2-10

In these examples, polyester yarn is separately spun and separately drawn. Polyester chips are dried and the intrinsic viscosity is ascertained. The viscosity is determined using a solution 40% by weight tetrachloroethane, 60% by weight of phenol, measured at 25° C. using 1.28% by weight of polyester, intrinsic viscosity then being determined as described in Example 1.

Chips are spun by melting in an extruder maintained under positive pressure and exited from the extruder through conventional filter media, then through a conventional spinnerette. The spun yarn then passes through

TABLE I  
Finish Component (All Values, Percent by Weight of Total Solids)

| Finish identity--percent solids finish                                                  | A 35 | B 35 | C 35 | D 35 | E 35 | F 35 | G 35 | H 35 | I 35 | J 35 | K 35 | HLB calculated values | Loss at 23° C. after 4 hours, percent | Physical state at room temperature |
|-----------------------------------------------------------------------------------------|------|------|------|------|------|------|------|------|------|------|------|-----------------------|---------------------------------------|------------------------------------|
| Concentration in the emulsion                                                           |      |      |      |      |      |      |      |      |      |      |      |                       |                                       |                                    |
| Lubricants, percent of total solids:                                                    |      |      |      |      |      |      |      |      |      |      |      |                       |                                       |                                    |
| Hexadecyl (isooctyl) stearate                                                           | 65   | 63.7 | 53.0 | 53   | 65   | 0    | 31   | 33   | 0    |      |      |                       |                                       | 2 Liquid.                          |
| Rearranged triglyceride                                                                 |      |      |      |      |      | 70   | 36   | 32   |      |      |      |                       |                                       | Do.                                |
| Emulsification agents:                                                                  |      |      |      |      |      |      |      |      |      |      |      |                       |                                       |                                    |
| Decaglycerol tetraoleate                                                                | 5.0  | 4.9  | 7.0  | (1)  | 15   | 15   | (2)  | 5.0  | (3)  |      |      | 6.0                   | 12.5                                  | Do.                                |
| Glycerol monoleate                                                                      | 6.0  | 5.9  | 9.0  | (1)  |      |      | (2)  | 6.0  | (3)  |      |      | 3.0                   | 16                                    | Do.                                |
| Ethoxylated tall oil fatty acid plus (15 E.O.)                                          |      |      |      |      |      |      |      |      |      |      |      |                       |                                       |                                    |
| Weighted average, HLB                                                                   | 8.0  | 7.8  | 11.0 | (1)  | 15   | 15   | (2)  | 8.0  | (3)  |      |      | 10.0                  | 5                                     | Do.                                |
| Weight of lubricant HLB ratio                                                           | 6.7  | 7.7  | 7.6  | (1)  | 7.6  | 8.0  | (2)  | 6.7  | (3)  |      |      |                       |                                       |                                    |
| Antistats and wetting agents:                                                           |      |      |      |      |      |      |      |      |      |      |      |                       |                                       |                                    |
| Sulfated glycerol trioleate                                                             | 4.4  | 4.9  | 4.1  | (1)  | 5.2  | 5.6  | (2)  | 4.4  | (3)  |      |      |                       |                                       |                                    |
| Ethoxylated alkylamine (20 E.O.)                                                        | 12.0 | 11.8 | 15.0 | (1)  |      |      | (2)  | 12.0 | (3)  |      |      | 14.0                  |                                       | Do.                                |
| Ethoxylated octyl phenol (12 E.O.)                                                      | 4.0  | 3.9  | 5.0  | (1)  |      |      | (2)  | 4.0  | (3)  |      |      | 15.5                  |                                       | Do.                                |
| Weight, percent HLB of antistats present                                                |      |      |      |      |      |      |      |      |      |      |      |                       | 12                                    | Do.                                |
| Antioxidants:                                                                           |      |      |      |      |      |      |      |      |      |      |      |                       |                                       |                                    |
| 4,4 thio-bis (6-tert-butyl-m-cresol)                                                    | 2.0  |      |      |      |      |      | (2)  |      | (3)  |      |      |                       |                                       |                                    |
| Emulsion stability                                                                      | 4E   | 4E   | Good | Fair | Good | Fair | Fair | 4E   | 4S   |      |      |                       |                                       |                                    |
| Overall average, HLB x weight percent lubricating agent/100 (lubricant agent HLB ratio) | 6.8  | 6.9  | 5.6  |      |      |      | 5.4  | 5.6  |      | 6.7  |      |                       |                                       |                                    |

<sup>1</sup> 47% sulfated esters of glycerols and ethoxylated esters of glycerides.<sup>2</sup> A mixture of 33% of sulfated esters of glycerides and ethoxylated esters or glycerides.<sup>3</sup> 100% mixture of ethoxylated glycerides and esters and may contain ethoxylated long-chain alkyl phenols.<sup>4</sup> E=Excellent.<sup>5</sup> S=Solution.

Table I shows a series of finishes which are evaluated at a 35% solids concentrate and 65% water concentrate level. On dilution, the emulsion viscosities are also determined under the same conditions as that used in determination of the concentrate as described above. In all cases, the emulsions are 35% solids and 65% water.

Table II shows the concentrate and emulsion viscosities in centipoises and wetting abilities in degrees of contact angle as well as the emulsion stability of the emulsions made up and illustrated in Table I. From Table II, it can be observed in general where low concentrate viscosities and low emulsion viscosities are obtained, the emulsion stabilities are excellent. However, where hexadecyl stearate is not included in the composition as illustrated by composition F, the emulsion stability is poor, even though the concentrate viscosity and the emulsion viscosity are low.

The wetting ability is measured in degrees of constant angle of a drop of each finish on a polyester film 75

60 a heated zone and passes through essentially quiescent countercurrent quench zones. The yarn exits from the quench zone and the filaments are guided uniformly over a textile fluid finish treatment roll.

After passing over the finish roll, the yarn passes through a guide to provide uniform spreading on the finish roll, thence to a take-up roll.

65 Table III gives the drawn yarn properties and drawing performance. The same finish compositions as indicated in Tables I and II are applied under identical circumstances. The results are shown in Table III.

70 From Table III, it can be observed that those finish emulsions which have excellent stability and a HLB ratio of  $6.8 \pm 4$  give excellent results in their drawing performance, good results on their yarn properties, excellent yarn-to-metal frictional properties, good slip stick properties, and very low static characteristics. None of the other finish compositions show equivalent overall good performance.

TABLE III

| Finish identity                                              | A          | B          | C      | D              | E          | F          | G            | H         | I         |
|--------------------------------------------------------------|------------|------------|--------|----------------|------------|------------|--------------|-----------|-----------|
| Example number                                               | 2          | 3          | 4      | 5              | 6          | 7          | 8            | 9         | 10        |
| Emulsion, percent solids                                     | 35         | 35         | 35     | 35             | 35         | 35         | 35           | 35        | 20        |
| Emulsion stability at 35% solids.                            |            |            |        |                |            |            |              |           |           |
| Manufacturing performance:                                   |            |            |        |                |            |            |              |           |           |
| Breaks per pound                                             | .00        | .00        | .03    | .04            | .00        | .03        | .02          | .00       | .32       |
| Wraps per pound                                              | .04        | .05        | .06    | .42            | .26        | .24        | .10          | .05       | .68       |
| Sum of the breaks and wraps/lb                               | .04        | .05        | .09    | .46            | .26        | .27        | .12          | .05       | 1.00      |
| Yarn deposit on the draw heater                              | Negligible | Negligible | Slight | Heavy deposits | Negligible | Negligible | Poor         | Heavy.    |           |
| Drawing performance:                                         |            |            |        |                |            |            |              |           |           |
| Yarn properties:                                             |            |            |        |                |            |            |              |           |           |
| Ultimate tensile strength, g./d.                             | 8.7        | 8.7        | 8.7    | 8.4            | 8.6        | 8.3        | 8.6          | 8.6       | 7.8       |
| Ultimate elongation 1/2%:                                    | 12.4       | 12.0       | 13.2   | 12.6           | 12.7       | 12.6       | 12.6         | 12.0      | 11.7      |
| Toughness index, $T_{TB}$ *                                  | 30.8       | 30.2       | 30.2   | 30.4           | 30.6       | 30.2       | 30.2         | 30.3      | 26.7      |
| Overall rating on yarn properties                            | Good       | Good       | Good   | Good           | Good       | Fair       | Fair to good | Excellent | Very bad. |
| Yarn-to-metal friction, gms.                                 | 213        | 228        | 268    | 305            | 290        | 284        | 293          | 216       | 314       |
| Yarn-to-yarn slip-stick friction:                            |            |            |        |                |            |            |              |           |           |
| Low                                                          | 146        | 175        | 178    | 160            | 152        | 108        | 165          | 137       |           |
| High                                                         | 633        | 646        | 632    | 647            | 647        | 615        | 542          | 566       |           |
| Static in millivolts                                         |            |            |        |                |            |            |              |           |           |
| Overall rating on frictional properties                      | 2          | 2          | 2      | 2              | 2          | 22         | 12           | 2         | 20        |
| Overall lubricity (HLB) ratio/denier of drawn yarn 1300/1322 | Excellent  | Fair       | Poor   | Fair           | Fair       | Poor       | Fair to good | Excellent | Poor.     |

Note.—Ultimate tensile strength in gms./den.  
\* Percent ultimate elongation.

The yarn-to-yarn method for testing of slip stick friction is described by Schlatter, Olney and Baer in the Textile Research Journal, vol. 29, pp. 200-210, March 1959. Briefly, the yarn interfilament frictional forces are determined by using a brush tension analyzer, Model ED-13-403, Brush Electronics Company, Cleveland, Ohio, wherein the yarn to be tested is passed at a speed of 1 cm./min. over pulleys, positioned so that the 2 strands under test, are twisted 1½ turns, and run against each other at an imposed helix angle of 360° with a positive tension of 600 grams. The frictional forces imposed are measured on a strain gage apparatus and recorded on a continuous recording chart. The chart frictional pattern shows a gradual increase in tension until the static friction is overcome. Then a rapid drop in tension occurs until a level is reached where the dynamic friction overcomes this imposed tension. Thus, the chart reads in a zig-zag pattern showing a continuous drop and rise in friction. Hence, the name slip stick friction. The high "slip stick" friction is a point in which static friction is overcome, or the frictional forces of the yarn evaluated with different finishes employed in this invention with the low level being the point where the dynamic frictional forces are overcome.

The yarn prepared in accordance with the present invention also demonstrates reduced yarn-to-metal frictional properties as compared with other finish compositions. The yarns showing excellent performance have a yarn-to-metal frictional property below 240 grams. Yarn-to-metal frictional force as referred to herein is determined in a manner as described by Schlatter in the same Textile Research Journal article as that described above in reference to yarn-to-metal interfilament frictional forces. The same brush tension analyzer is employed and the yarn is passed at a speed of 1000 ft./min. with one turn over a chromplated polished, stainless steel pin ¼" diam. of surface finish of root mean square of 2.5 microinches giving a metal-to-yarn angle of 360° against a floating pretension rate of 20 grams. The chart reading shows the constant tension which is a measurement of the yarn-to-metal frictional forces. The static is measured by the following method.

The same brush tension analyzer is employed and the yarn is passed through a Faraday Eye placed right after the stainless steel pin, which is induced by the static created on the pin by the yarns friction during the yarn to metal frictional test.

A Faraday Eye consists of two concentric copper tubes insulated and having a 3 mm. diameter hole perpendicular to the tubes. The static electricity transmitted to the Faraday Eye by induction is connected in series to an electrometer-amplifier-recorder system where the static reading is taken.

#### Examples 11, 12, 13

The tire yarns from Examples 2, 3, and 8, are compared with a known tire yarn having exceptionally good properties. The yarn is twisted in an 8/8 turns/in. construction. All yarns listed in Table IV are twisted in one direction for 8 turns and then the 3 ends of 1300 denier are cabled together by twisting 8 turns in the opposite direction.

The cords are predipped in a toluene diisocyanate solution that contains para-, ortho- and meta mixtures. The materials are then passed through a rubber-latex<sup>1</sup> resorcinol formaldehyde finish of the following composition.

|                                                          | Parts by weight |
|----------------------------------------------------------|-----------------|
| Rubber latex                                             | 244             |
| Resorcinol                                               | 11              |
| Formaldehyde                                             | 16.2            |
| Water                                                    | 298.5           |
| Sodium hydroxide                                         | .3              |
| <sup>1</sup> Butadiene-styrene-vinylpyridine-terpolymer. |                 |

The yarn is tensilized for a 2% stretch at a temperature of 450° F. on a Litzler tensilization unit.

## 11

Two samples of cord are prepared from each tire yarn and the results of their values are cited as an average of 2 separately prepared cords and separately tested cords. The results of these tests are cited in Table IV.

Referring to Table IV, Examples 11 and 12, the textile fluid finish composition of this invention yields tire cord of superior strength and toughness index and superior final breaking strength. The adhesion and the flexural fatigue tests show yarn containing the finish compositions of this invention to be superior to other finish types and to known commercial yarns. Wheel durability tests show the yarn at least equal to or perhaps slightly superior to commercial polyester yarn and with a commercial finish composition employed as a control.

TABLE IV  
Cord Construction (3 Ends of 1,300 Denier Twist 8/8)

| Finish composition identity                                                                   | A     | B     | G     | Commercial<br>yarn and<br>finish |
|-----------------------------------------------------------------------------------------------|-------|-------|-------|----------------------------------|
| Yarn identity Example No.                                                                     | 2     | 3     | 8     |                                  |
| Dipped tensilized cord properties                                                             | 11    | 12    | 13    | Control                          |
| Cord breaking strength, lbs                                                                   | 60    | 60.75 | 57.6  | 62.2                             |
| Cord elongation at break                                                                      | 19.9  | 20.7  | 19.25 | 20.3                             |
| Cord toughness factor of cord<br>elongation $\frac{1}{2} \times$ lbs. breaking<br>strength/10 | 26.8  | 27.7  | 25.3  | 27.8                             |
| Cable twist dipped cord                                                                       | 8.30  | 8.30  | 8.33  | 7.86                             |
| Load at 10% elongation, lbs                                                                   |       |       |       |                                  |
| Heat shrinkage:                                                                               |       |       |       |                                  |
| 1 hour at 350° F, percent                                                                     | 5.45  | 5.15  | 5.05  |                                  |
| $\frac{1}{2}$ hour at room temperature,<br>percent                                            | 5.15  | 4.95  | 4.8   |                                  |
| Thermal stability:                                                                            |       |       |       |                                  |
| Final break strength, lbs                                                                     | 44.05 | 43.6  | 41.8  |                                  |
| Adhesion U test <sup>3</sup>                                                                  | 105   | 105   | 100   | 100                              |
| Flexure fatigue rating <sup>1</sup>                                                           |       |       |       |                                  |
| Goodyear tube test                                                                            | 115   | 105   | 102.5 | 100                              |
| Wheel tests, tire durability,<br>hrs. <sup>2</sup>                                            | 51    | 47    |       | 45-50                            |

<sup>1</sup> ASTM Standard, 1964, part 25, pages 205-208, at 50 p.s.i. pressure in the tube. Commercial yarns typical rated at 100.

<sup>2</sup> Wheel test durability. The single-end tires were prepared in a conventional manner from the above tire cords. A 8.25 x 14/2 ply/tire was inflated to 24 p.s.i. tire run at 60 miles per hour, 7 hours, 1,210 pounds; 7-16 hours at 1,450 pounds; and after 16 hours, ran to failure at 1,690-pound load.

<sup>3</sup> Similar to test method described in U.S. Pat. 3,369,057, Feb. 13, 1968, page 10, lines 1-17—Commercial polyester tire yarn rated at 100.

## Example 14

Polyester chips of the same quality as employed for Examples 2 through 10 are spun in a continuous operation and are drawn to produce a drawn industrial yarn. The yarn has an ultimate tensile strength of 8.5 gms. per denier and an elongation of 13%. The yarn is drawn. As in the first case, 0.7% finish was applied from a 35% aqueous emulsion using the same textile fluid finish composition as indicated by A-I in Table I. The polyester was drawn.

Yarns from finish composition A, B and H gave satisfactory and uniform drawing performance. Yarn with finish composition C and E spun and drew only fair. However, yarns containing finish compositions of D, F, G, and I drew so poorly that they could not be strung up at normal speeds.

## Example 15

In place of polyester, polycaproamide fibers having a formic acid viscosity of 60 are passed over a draw pin and then over a heater, then over a draw roll, then over a winder. The yarn is then drawn.

## 12

Polycaproamide yarns coated with finish compositions A, B, C and H gave excellent performance. Yarns containing finish compositions C and E gave respectively fair and good performance, whereas yarns D, F, G, and I gave poor performance in the same general pattern as that obtained for the polyesters illustrated in Examples 2 through 10.

## Example 16

In this example, textile fluid finish compositions A-I of Example 1, the 65 weight percent of water was replaced with a low viscosity fluid, tetraethylene glycol di(2-methyl hexoate). The industrial yarn is spin-drawn as in Example 14 with again improved performance for A, B, E and H and somewhat inferior drawing performance and strength properties in C, D, F, G, and I. Other additives suitable for use in the present invention in lieu of the aqueous make-up are kerosene, triethylene glycol dipelargonate, neopentylglycol dipelargonate, octyl-decyl adipate, diisooctyl azelate, diethyl hexyl sebacate.

It is claimed:

1. Synthetic polyester filamentary yarn comprised of filaments which are treated with from about 0.4 to about 1.5 weight percent based on the weight of the yarn of a liquid composition consisting essentially of an emulsifying agent comprising about 4.9 to about 5.0 weight percent of said composition of decaglycerol tetraoleate, about 5.9 to about 6.0 weight percent of said composition of glycerol monooleate, and about 7.8 to about 8.0 weight percent of said composition of ethoxylated tall oil fatty acid, an antistat and wetting agent comprising about 11.8 to about 12.0 weight percent of said composition of sulfated glycerol trioleate, and about 3.9 to about 4.0 weight percent of said composition of an ethoxylated alkylamine and a lubricant of about 55.0 to about 75.0 weight percent of said composition hexadecyl stearate.

2. The yarn of claim 1 wherein the treating materials have an additional ingredient of about 1.0 to about 5.0 weight percent of said composition of an antioxidant consisting of 4,4'-thiobis-(6-tert-butyl-m-cresol).

3. The yarn of claim 1 wherein the lubricant comprises about 30.0 to about 35.0 weight percent of said composition of hexadecyl stearate and about 30.0 to about 35.0 weight percent of said composition of rearranged triglyceride.

## References Cited

## UNITED STATES PATENTS

|           |          |                |           |    |
|-----------|----------|----------------|-----------|----|
| 3,563,892 | 1/2/1971 | Cooley         | 117—138.8 | X  |
| 3,224,889 | 12/1965  | Schulde et al. | 117—139.5 | CO |
| 3,296,019 | 1/1967   | Keller et al.  | 252—8.8   |    |
| 3,306,850 | 2/1967   | Olsen          | 252—8.9   |    |
| 3,428,560 | 2/1969   | Olsen          | 252—8.9   |    |
| 3,470,095 | 9/1969   | Pontelandolfo  | 252—8.6   |    |

WILLIAM D. MARTIN, Primary Examiner

S. L. CHILDS, Assistant Examiner

U.S. Cl. X.R.

117—139.5 CQ; 252—8.6, 8.75, 8.9